

# UNITED STATES PATENT OFFICE.

JOHN J. BOERICKE, OF MERION, PENNSYLVANIA.

## METHOD OF PRODUCING METALS.

1,277,035.

Specification of Letters Patent. Patented Aug. 27, 1918.

No Drawing. Application filed July 20, 1914, Serial No. 851,886. Renewed June 29, 1918. Serial No. 242,865.

*To all whom it may concern:*

Be it known that I, JOHN J. BOERICKE, a citizen of the United States, residing at Merion, in the county of Montgomery and State of Pennsylvania, have invented certain new and useful Improvements in Methods of Producing Metals, of which the following is a specification.

This invention relates to the reduction of metals, particularly rarer metals, such for example, as vanadium, chromium, manganese, and the like, by what is known as the alumino-thermic process, wherein metallic aluminum, a mixture of aluminum or an alloy of aluminum, or other material having an affinity for oxygen, is used as the reducing agent. The primary object of my invention is the provision of an improved method whereby the rarer metals can be produced very economically and the comparative yield of and the quality of the finished product greatly increased and improved.

The foregoing, together with such other objects as may hereinafter appear, or are incident to my invention, I attain by means of an improved method which will be fully described.

It has long been known that metallic aluminum is a powerful agent in reducing ores, and it has also been known that when the aluminum used is in a very finely pulverized condition, the reaction between the aluminum and the oxids, sulfids or chlorids, as the case may be, if started in a portion of the mixture, will continue throughout the mass; in other words, an exothermic reaction takes place. Because of the fact that aluminum is an expensive reducing agent, its application has been limited to the production of metals and alloys of comparatively high value. The cost of production has been large not only because of the fact that it was considered necessary to finely pulverize the aluminum, but also because the metallic ores or compounds from which the desired metal was to be reduced were likewise pulverized in carrying out the known processes. As previously stated, it is one of the chief objects of my invention to reduce the cost of production not only by making the process less expensive, but also by improving and increasing the yield and the quality of the finished product.

In carrying out my improved method, I have discovered that in place of the finely

pulverized aluminum heretofore used in the art, aluminum in the form of ingots can be employed. Aluminum in ingot form is only slightly more expensive than the ordinary 60 ingot aluminum which is the cheapest commercial form in which aluminum is sold. In the practice of my invention, I prefer to employ ingot aluminum of which the ingots or lumps vary in size from in the neighborhood of one-eighth of an inch in diameter, to three-quarters of an inch, or an inch in diameter. Ingot aluminum is aluminum in solid, lump form and may include granular ingot aluminum which is also in solid, lump 70 form, but is usually made by dropping the hot metal into water, thus forming what is ordinarily termed shot, the dimensions of which may vary considerably.

It will be understood that the aluminum 75 is mixed with the ore or compounds in a crucible or other vessel in any desired proportion, and a reaction started, preferably by igniting a portion of the mixture from which the reaction spreads throughout the 80 mass. Where ingots of aluminum are used, it is not necessary to pulverize the ores or compounds, and I prefer not to do so, as the finished product is somewhat improved in quality. It will of course be understood that 85 the ores are crushed before reduction, but according to my process it is not essential that they be pulverized.

In order to effect an additional saving in cost, as a preliminary step I prefer to pre- 90 heat the raw materials entering into the reaction, and such preheating may be done either before or after the mixing of the aluminum with the metallic compound. The reaction, however, should be instituted be- 95 fore the heated materials cool. I have found that this step results in a substantial in- 100 crease of yield, and it is particularly useful in reducing the oxids of the rarer metals, as, for example, in the manufacture of ferro- 105 vanadium. Another advantage incident to this step is that a saving is effected in the amount of aluminum required for the reduc- 110 ing operation. I have also found that my improved method secures superior results from low grade ores, that is, ores which contain only a small percentage of the rare metal to be reduced. In fact I have been able to reduce a superior product from ores hitherto regarded as useless. An additional 115 saving, as well as better results, are obtained by also preheating the crucible or other form

of container which is used to carry out the reduction.

My invention also contemplates an additional step tending to increase the quantity and quality of yield, and this step consists in subjecting the ores, just previous to their reduction, to the action of the atmosphere so as to insure complete oxidization. I prefer to take this step when preheating the ores at which time it can be readily done by simply opening the furnace doors to create a draft over the ore and then in stirring or agitating the ore. A large amount of oxygen is thus absorbed by the ore and I have found by experience that this step has a material effect on the resultant product.

It will be obvious that the method can be used not only to reduce metals, but also alloys.

20 I claim:

1. The herein described process of producing metals or alloys from metallic compounds which consists in mixing ingot aluminum with the compound and in instituting an exothermic reaction.

2. The herein described process of producing metals or alloys from metallic compounds which consists in preheating the compound, in mixing ingot aluminum with the compound, and then in instituting an exothermic reaction.

3. The herein described process of producing metals or alloys from metallic compounds which consists in mixing ingot aluminum with the compound, in preheating the mixture, and then in instituting an exothermic reaction.

4. The herein described process of producing metals or alloys from metallic compounds which consists in mixing ingot alu-

minum with the compound, in preheating the aluminum before admixture, and then in instituting exothermic reaction.

5. The herein described process of producing metals or alloys from metallic compounds which are not finely divided, which consists in mixing with the compound ingot aluminum, and then in instituting an exothermic reaction. 45

6. The herein described step of treating metallic compounds preparatory to reduction by the alumino-thermic process which consists in subjecting the compound by agitation to the action of the atmosphere to secure oxidization. 50

7. The herein described step of treating metallic compounds preparatory to reduction by the alumino-thermic process which consists in preheating the compound and subjecting it by agitation to the action of 55 the atmosphere to secure oxidization.

8. The herein described step of treating metallic compounds preparatory to reduction by the alumino-thermic process which consists in mixing a reducing agent in ingot 60 form with the compound to be reduced, and then in instituting an exothermic reaction.

9. The herein described step in producing metals or alloys from metallic compounds by the alumino-thermic process which consists in carrying out the reaction with aluminum in lump form. 70

In testimony whereof I have hereunto signed my name in the presence of the two subscribed witnesses.

JOHN J. BOERICKE.

Witnesses:

L. A. MYERS,  
ARTHUR SYNNESTVEDT.